

Feb. 20, 1945.

G. L. FISK

2,369,730

METHOD OF ROLLING METAL BARS

Filed June 12, 1942

4 Sheets-Sheet 1



*Fig. I.*



INVENTOR  
Gustaf L. Fisk  
by his attorneys  
Stebbins and Blenko



Feb. 20, 1945.

G. L. FISK

2,369,730

METHOD OF ROLLING METAL BARS

Filed June 12, 1942

4 Sheets-Sheet 2



INVENTOR  
Gustaf L. Fisk  
by his attorneys  
Stebbins and Blenko

Feb. 20, 1945.

G. L. FISK

2,369,730

METHOD OF ROLLING METAL BARS

Filed June 12, 1942

4 Sheets-Sheet 3



*Fig. 6.*



*Fig. 7.*



*Fig. 8.*



*Fig. 9.*



*Fig. 10.*



Feb. 20, 1945.

G. L. FISK

2,369,730

METHOD OF ROLLING METAL BARS

Filed June 12, 1942

4 Sheets-Sheet 4

*Fig. 14.*



*Fig. 15.*



*Fig. 15.*

*Fig. 16.*



*Fig. 17.*



INVENTOR  
Gustaf L. Fisk  
by his attorneys  
Stebbins and Bleke

## UNITED STATES PATENT OFFICE

2,369,730

## METHOD OF ROLLING METAL BARS

Gustaf L. Fisk, New Fairfield, Conn.

Application June 12, 1942, Serial No. 446,716

8 Claims. (Cl. 80—63)

This invention relates to the rolling of bars of a great variety of sections, commonly known as merchant bars and shapes, including bars of circular cross section, known as rounds, and particularly to a method whereby they may be finished to precise dimensions within close tolerances.

The round is perhaps the most common but also one of the more difficult sections to produce to accurate dimensions. The need and demand for accuracy in rounds are so pronounced and the problems involved in producing an accurate round have received so much attention in the trade, that I have chosen to explain my improved method of rolling with particular reference to this section.

Merchant bars have usually been made heretofore by hot-rolling to finished size. According to one method of rolling rounds, a billet is reduced by hot-rolling to an approximate round slightly larger than the desired finished size. It is then entered repeatedly by hand while still hot, into a finishing pass between a pair of rolls having grooves of circular section therein relieved at the parting, thus permitting slight side spread of the bar as it is rolled. For this reason, after the first finishing pass, the bar must be gripped to hold it in such position that the major axis of its section is perpendicular to the axes of the rolls. To this end, the operator grips the rear end of the bar with tongs when entering the lead end into the pass and follows the bar up to the mill as it is rolled, maintaining his tong grip thereon until the rear end of the bar enters the pass. This method limits the peripheral speed of the rolls to the speed at which the operator can walk and control the bar. Only short lengths of bar, furthermore, can conveniently be held against turning in the pass. Thus, while the method produces accurate products, the cost is prohibitive because of the low output.

According to another method of producing rounds, a billet is reduced to an approximate ellipse and entered into the finishing pass between side guides placed close to the pass. These guides enter the bar properly with the major axis of its section perpendicular to the axes of the rolls. This requires that the bar have a section with the major axis much greater than its minor axis and this in turn necessitates a considerable side spread in converting the elliptical section to a round in the finishing pass and the amount of such spread is subject to little control. Any slight change in size, shape or temperature along the length of the entering bar or

between successive bars will produce a considerable difference in the amount of side spread. As a result, the horizontal diameter of the bar as it leaves the finishing pass is characterized by excessive variations from the desired dimension. For these reasons, relatively large tolerances are permitted, viz., for a 1" round  $\pm .009"$ , and a maximum .013" out-of-round at any given point. The tolerances vary, of course, with the size of the bar.

The various factors which cause inaccuracy in the finished dimensions of rolled metal bars including that just explained, may be summarized as follows:

- 15 A. Misalignment of rolls and changes in pass area, principally due to bearing wear during the rolling operation. In the case of the more modern mills, however, these difficulties have been eliminated with the use of anti-friction radial and thrust bearings for the rolls and with rigs for micrometer roll adjustments.
- 20 B. Change in temperature from end to end of the bar, due to the longer exposure of its rear end prior to the finishing pass; temperature variations between different bars, due to mill delays; and temperature differentials due to improper heating. Naturally, the colder the metal in passage between the rolls, the greater the pressure on the rolls and the larger the section emerging from the pass. With improved furnace and mill design and practice, inaccuracies due to temperature fluctuations of the metal in process have been materially reduced but by no means eliminated.
- 25 C. Improper entry of bars into the roll passes, particularly at the finishing end of the mill, or to obtain proper entry, the delivery of a section to the finishing rolls, which cannot be duly controlled as to "side-spread" for accuracy of product.
- 30 Attempts have been made in the past, with more or less success, to reduce the inaccuracies due to uncertain side spread in rolling guide rounds, i. e., rounds rolled by introducing an elliptical bar into a finishing pass by side guides as above described. One such attempt calls for a separate finishing stand equipped with a pair of vertical rolls and, in immediate juxtaposition thereto, with a pair of horizontal rolls grooved to furnish the finishing pass. This stand is added beyond the last pair of rolls of the guide mill, at a suitable distance to permit the formation of a free loop between the rolls of the guide mill and the vertical rolls of the finishing stand.
- 35
- 40
- 45
- 50
- 55

signed to produce an approximate round in the last pass of the guide mill, convert it by continuous rolling into an ellipse in the vertical rolls of the finishing stand, and then instantly to change this elliptical section into a finished round in the horizontal rolls of the finishing stand. The minor axis of the ellipse being but slightly smaller and the major axis but slightly larger than the desired diameter of the finished round, the reductions in the rolls of the finishing stand are relatively slight, and the uncertain side spread correspondingly small. The approximate round and the ellipse cannot be held against axial turning in the passes of the finishing stand, but the very limited distance between the passes of the two sets of rolls is intended to preclude improper entry into the finishing pass. With any slight variation in size, shape or temperature, however, the hot bar in motion between the two passes of the finishing stand would be subject to serious variations of tension or compression or both, due to the close proximity of the two sets of rolls, resulting in serious fluctuations in sectional area of the finished bar. If the sets were separated, on the other hand, to allow for a loop or slack between the two roll passes, then proper entry of the ellipse into the finishing pass, could not be accomplished.

A better method for reducing the inaccuracies due to uncertain side spread calls for a stand of vertical rolls to furnish the final pass, beyond but in fairly close proximity to the last stand of the horizontal rolls of the guide mill. In this method, the bar is rolled to final size in the pass of the last stand of the guide mill, except that excess metal is forced into the roll cavities to concentrate all variations in sectional area, due to uncertain side spread into definite over-fills. The bar is then passed immediately between a pair of grooved vertical rolls. The object of the final pass in the vertical rolls is to eradicate the over-fills, as far as possible, to complete the round. The rolls are placed in line for straight delivery of the bar from the corresponding pass in the rolls of the last stand of the guide mill, and the guides immediately ahead of these guide-mill rolls, serve to hold the bar against axial turning. By aid of modern mill machinery, a skillful operator may thus roll within narrow tolerance limits. By way of example, 1" rounds may be rolled in this manner within a total variation of .005" in diameter and .003" out of round, but such accuracy cannot be maintained without sacrifice of output.

Cross-rolling of hot guide rounds, in special rolls, has been proposed to reduce their inaccuracies. Although this scheme is entirely feasible, it has little practical value due to the strictly limited speed of the cross-rolling process.

The inaccuracies of hot-rolled bars may also be reduced by cold working. Cross rolls serve to improve the roundness and surface of cold bars and, under certain conditions as to angular position and shape of rolls, may also serve to reduce their sectional area. Cold drawing, through dies in draw-benches, is a common and dependable way to produce bars of superior accuracy. By way of example, 1" rounds may be drawn in this manner within a total variation of as little as .001" in diameter.

Except for the field of wire drawing, by aid of dies and blocks, the present cold working methods are limited to short lengths and are slow and expensive as compared to hot rolling. On the other hand, they furnish not only su-

perior accuracy, but cold working also improves the surface and (cold drawing in particular) the physical properties of rolled products.

It is one of the purposes of my invention to obtain the advantages of cold drawing by a new and economical method of cold rolling long lengths at high speed in conjunction with a hot mill, but without restricting the hot mill as to output or accuracy beyond those of the ordinary tonnage mill.

It is a further object of my invention to remove the inaccuracies characterizing hot rolled bars by eliminating variations in the temperature of the bar as it progresses through the final passes and by insuring proper entry and control of side spread in these passes.

In a preferred practice of my invention, I roll a rough round on a guide mill having its last pass shaped to give the bar a slightly oval shape, i. e., round with overfills on opposite sides, and a size greater than that desired in the final product. After the hot-roller bar has cooled to a temperature below the recrystallization temperature, preferably on a pack-annealing cooling bed, I subject the bars to cold rolling in a tandem cold mill having two or more passes, the rolls of the several stands being so driven as to tension the portion of the bar between adjacent stands. The combined effect of the tensioning and cold rolling is to reduce the rough rounds to finished bars having the desired size and shape within very close tolerances.

A more complete understanding of the invention and the advantages thereof may be gained from the following detailed description and explanation which refer to the accompanying drawings illustrating diagrammatically the preferred practice of the invention. In the drawings,

40 Figure 1 is a partial section through the rolls of the last stand of a hot mill for producing a rough round adapted to be finished according to my invention;

45 Figure 2 is a diagrammatic plan view illustrating one mode of applying the invention;

Figures 3 and 4 are partial sections through the rolls of the stands of the mill of Figure 2 showing the shape of the passes therebetween;

50 Figure 5 is a view similar to Figure 1 illustrating a modified practice;

Figure 6 is a diagrammatic plan view of the mill utilized in the modified practice;

Figures 7 through 10 are views similar to Figures 3 and 4 showing the shape of the passes between the rolls of the several stands of the mill of Figure 6;

Figure 11 is a diagrammatic layout of a mill adapted to carry out the invention;

Figures 12—A and 12—B together constitute a modified mill layout;

Figure 13 is a diagrammatic plan view illustrating a modification of my invention adapted for effecting a heavy cold reduction of a hot-rolled bar to produce a cold-rolled bar of much smaller size for further processing;

Figure 14 is a partial sectional view taken on the plane of line XIV—XIV of Figure 13, and

Figures 15 through 18 are views similar to Figures 3 and 4 showing the shapes and relative sizes of the passes between the rolls of the several stands of the mill of Figure 13.

A preferred practice of my new method for removing the inaccuracies of hot-rolled rough rounds will be explained with particular reference for the present to Figures 1 through 4. As

shown in Figure 2. I subject the hot-rolled bars, after they have cooled to a temperature below the recrystallization temperature, to cold-rolling in a 2-stand, tandem cold mill 1. This cold mill comprises a stand of horizontal rolls 2 and a stand of vertical rolls 3. The rolls of both stands are driven, in the customary manner by an individual motor, and are grooved for a series of roll passes. For the sake of clarity, only one pass is shown in each pair of rolls; that is, pass 4 in the horizontal rolls and the corresponding pass 5 in the vertical rolls. These passes are shown in detail in Figures 3 and 4. A bar in passing through the cold mill, follows a fixed and straight pass line and the horizontal and the vertical rolls are made adjustable in the longitudinal direction to bring any desired pass into alignment with the pass line. The two sets of rolls are placed in close proximity to one another, say on 2' centers, and with this purpose in view, the horizontal and the vertical rolls are preferably mounted in a common housing.

The cold mill rolls are journaled in anti-friction bearings for radial and thrust loads and micrometer roll adjustments may be provided, to eliminate inaccuracies in mill products due to bearing wear or misalignment of rolls. Since the products are rolled cold, inaccuracies due to temperature variations of the metal in process are also eliminated. Proper entry into the roll passes and control or elimination of side spread, are accomplished in the manner now to be set forth.

To produce a cold rolled round such as shown in finishing pass 5, a rough round B of somewhat larger diameter is first produced in a stand 6 of the hot mill, having a pass 6a shown in Figure 1. By way of example, if it be desired to cold roll a 1" round and the hot mill can readily roll within a total tolerance of .020", then the rough round may be produced varying in diameter within 1.010" to 1.030", except when measured horizontally as it emerges from the pass. In that direction the dimensions will preferably be made greater by forcing metal into the roll cavities 7 to produce over-fills 8 and give the rough round a definite major axis.

The hot-rolled bars are delivered to any convenient form of cooling bed by a suitable run-out conveyor, and preferably to a pack-annealing cooling bed for slow cooling below the recrystallization temperature prior to finishing by cold rolling. Suitable arrangements of conveyors, cooling beds and associated apparatus are shown in Figures 11, 12-A and 12-B and will be described in detail later.

Referring now to the cold mill 1, the rough round after cooling is entered into the pass 4 of the horizontal rolls with its major axis horizontal, thus preventing the bar from turning in the pass by allowing it to take the path of least resistance. Since the finishing pass 5 in the vertical rolls is in strict alignment with pass 4 in the horizontal rolls, since the two sets of rolls are in close proximity to one another, and since the cold bar has the necessary stiffness in passing from the rolls 2 to the rolls 3, proper entry into the finishing pass 5 is assured. The proper entry of the rough round into the pass 4 of the horizontal rolls 2 of the cold mill is facilitated by the tendency of the bar to lie with its major axis in horizontal position. Furthermore, the over-fills 8 will be plainly visible to the operator in that the metal there will be less smooth than where it contacted the rolls in the final pass of the hot mill. The rough round, preparatory to entry

into the cold mill, rests freely on a cold mill approach table and can be turned by the operator, by aid of a pair of tongs, as required for exact entry in feeding the bar to the mill.

5 The section of rough round B is shown by dot-and-dash arcs in Figure 3 in relation to pass 4 to indicate the draft 9 in the horizontal rolls 2 of the cold mill. The draft 10 in the finishing pass 5 of the vertical rolls 3 is also illustrated in 10 Figure 4 where the dot-and-dash arcs indicate the section of the bar after traversing pass 4. It will be noted that the bar is rolled to finished height in the horizontal rolls 2 and that no side spread is permitted by the final pass 5 in the vertical rolls.

15 I eliminate or control side spread in the passes of the cold mill by maintaining the metal under controlled tension during cold rolling. If the bar be subjected to sufficient pull in longitudinal direction, then the reductions in the roll passes will cause the metal to elongate in the direction of pull rather than spread in directions at right angles thereto. Furthermore, if the reduction be made proportionate throughout the section, then all the metal will tend to flow in the direction of pull, to take the shape of the pass, without side spread. Thus my new process is, in effect, a combination of rolling and drawing between rolling dies.

20 30 The desired tension in the bar is maintained in the distance between the horizontal and the vertical rolls of the cold mill, by the use of motors of suitable characteristics to drive the respective sets of rolls. The tension is controlled 35 by controlling the relative speeds of the motors. The electrical equipment required to achieve this result is well known and requires no detailed disclosure. Only its functions will be briefly referred to in explaining my preferred method of 40 operation.

45 When the rough round B is fed to the cold mill, the horizontal rolls 2 are run at relatively slow speed. The vertical rolls 3 are operated at a somewhat higher speed, to compensate for the reduction in the pass 5 and to produce desired pull on the bar when its front end enters the 50 pass 5. At that instant, the increased load on the motor driving the vertical rolls 3 causes a load relay to function so as to automatically increase the speed of rolls 2 and 3, while maintaining the tension in the bar unchanged. The excess speed of rolls 3 results in a pull on the bar, by forcing their motor to also take part of the load on rolls 2, to cause their corresponding increase 55 in speed. In other words, the rolls 2 and their motor furnish a drag on the bar, adjustable by motor speed control. As the rear end of the bar is nearing the pass 4, a flag switch or other suitable device functions to automatically and progressively reduce the speed of the rolls 2 and 3. The purpose is to cause the bar, now in motion at high speed, to exert a limited pull on the rolls 3 and thus continue the metal under tension in 60 pass 5, while the rear end of the bar travels the distance, in whole or part, from pass 4 to pass 5. The momentum of the bar is thus utilized to maintain a limited tension as its rear end leaves and travels beyond the horizontal rolls 2. The speed of the rolls is reduced in this way to the 65 suitable speed of entry, the next rough round is fed to the cold mill and the process is repeated. As to the rate of rolling, two cold mills 1 will usually keep pace with the production of the hot mill.

70 75 The front end of the bar is not subject to ten-

sion while it covers the distance from pass 4 to pass 5. To compensate, the draft 9 is purposely made small as compared to draft 10 and the rolls 2 are shaped to form cavities 11 to allow for the correspondingly small side spread at the front end of the bar in pass 4. Furthermore, this slight side spread is distributed over wide areas, where the bar does not contact the rolls 2, and is thus made small enough so that any effect on the accuracy of the bar is practically eliminated under tension in the succeeding pass 5. During the short interval when the end of the bar is passing through the rolls 2 without benefit of tension, the speed of rolling is relatively low so the power input is not unduly high, the lack of tension notwithstanding.

It should be noted in this connection that the tension serves to materially reduce the power required for the pass reductions. It also eliminates chances for compression of the metal in the bar between adjacent stands, which would cause variations in size of finished bar.

Due to the absence of temperature fluctuations of the metal in process, the variations in the pressure on the rolls will be due to the limited variations in size of the rough rounds, and will cause but slight deviations in the deflection of the rolls in the cold mill. By way of example, the 1" rough round above referred to, if made of soft steel and finished by cold rolling in the manner specified above, and using rolls of a size ordinarily used in the finishing end of the hot mill, would vary in diameter, due to roll deflection, much less than .001". It is thus entirely feasible, in case of 1" rounds used as an example, to roll within a total tolerance variation of as little as .001" in diameter, except possibly for the extreme ends of the rolled lengths.

By removing the causes of inaccuracy in rolling metal bars, as explained in preceding paragraphs, my new process permits the rolling of merchant bars and shapes within cold drawn tolerances. The cold rolling operation, preferably done in conjunction with the hot mill, in no way limits or interferes with the operation of the hot mill. The cold mills roll annealed bars, using the cooling bed lengths produced on the hot mill, and have sufficient finishing capacity to keep pace with the hot mill. 2-high rolls furnish the necessary stiffness for the cold rolling required in finishing bars of ordinary size and hardness, and the cost of the extra equipment needed to practice the new process is relatively small when compared to the total cost of the complete hot mill. The cold rolling is accomplished with a minimum of handling and the extra labor involved is a minor item when compared to the total labor force on the complete mill. All of these factors, combining high production and low cost with superior accuracy, make for quality and economy not attainable by any hitherto known process.

In case of products requiring a bright finish, it is necessary to free the bars from scale, by pickling, prior to cold rolling. In this connection, the desired surface hardness and physical properties may be imparted to the bars by controlling the amount of cold working. Without resorting to 4-high rolls, which would be expensive and complicated, considerable reductions can be made in the passes of the 2-high cold mill without loss of accuracy, particularly on the smaller bar sizes. Naturally, the narrower the section, the smaller the pressure on the rolls and the larger the draft that can be taken on 2-high rolls. For this pur-

pose, I use a cold mill 12 shown in plan view in Fig. 6. Each stand of rolls is driven by an individual motor and is grooved for a series of roll passes. For the sake of clarity, only one pass is shown in each pair of rolls. By way of example, the passes 13, 14, 15 and 16 to produce a round are shown in detail in Figures 7 through 10. A bar, in passing through the cold mill, follows a fixed and straight pass line and the horizontal and the vertical rolls are made adjustable in longitudinal direction to bring any desired pass into alignment with the pass line. The four sets of rolls are placed in close proximity to one another, say on 2' centers, and with this purpose in view, they are preferably mounted in a common housing.

To produce a cold-rolled round such as shown in finishing pass 16, a blank of larger diameter, to allow for required cold working, is first produced in the hot mill. The final pass 17 in the hot mill, is illustrated in Figure 5 and provides for roll cavities 18. The blank 19 is preferably rolled with pronounced over-fills 20, to give it a definite major axis. Proper entry into the several passes of the cold mill is then accomplished in the manner already described with reference to cold mill 1.

The passes 13 through 16 are designed to eliminate side spread by maintaining the metal in process under controlled tension. The desired tension loads on the bar are established in the distances separating the several sets of rolls, by aid of motor and electric control equipment, such as already referred to in connection with cold mill 1.

When the blank 19 is fed to the cold mill, the first set of horizontal rolls 13' are run at relatively slow speed. The succeeding sets of rolls 14', 15' and 16' are operated at progressively higher speeds to compensate for the drafts in passes 14, 15 and 16 and to produce the various desired pulls on the bar. When the front end of the bar enters the pass 14, the speed of all the rolls is automatically increased, to speed the rolling operation, while maintaining the established tension loads on the bar unchanged. As the rear end of the bar is nearing the pass 15, the speed of all the rolls is automatically and progressively reduced, at a rate to utilize the momentum of the bar to maintain a limited tension on the metal in the finishing pass 16, as its rear end leaves and travels beyond the pass 15. Practically the entire length of bar can thus be rolled under tension in all the passes of the cold mill, except for the front end, while it covers the distance from pass 13 to pass 14. This situation is compensated for in the way already explained with reference to cold mill 1. As to the rate of rolling, two cold mills 12 are preferably used to keep pace with the hot mill.

By way of example,  $\frac{1}{2}$ " rounds of desirable physical properties and of superior accuracy and surface, may thus be rolled from  $\frac{3}{4}$ " blanks of soft steel, in 2-high rolls journaled in anti-friction bearings. Because of the tension maintained in the metal during the cold rolling process, the motor horse-power requirements and the power consumption are relatively small.

A mill layout for practicing my invention is shown in Figure 11. In it, 21 represents the last set of rolls in a guide mill, of any suitable construction and arrangement, for hot rolling of merchant bars and shapes, including rounds. The hot rolled products are delivered by run-in tables 22 to position for handling by the mech-

anisms of a double cooling bed 23. This bed, ordinarily 250 ft. or more, in length, to accommodate the rolled lengths, is of the pack-annealing type. In other words, it is equipped for slow cooling of the hot bars in contact with one another. Such cooling beds have been on the market for a number of years, available for annealing of rounds, squares, flats and other sections, but they have been used principally for the annealing of spring flats. One of the objects of my invention is to utilize the advantages of such beds, not only for annealing of spring steels and the like, but also for the production of soft metal bars of superior accuracy, surface and physical properties.

The run-out tables 24, from the cooling bed, lead to crop shears 25, and run-out extension tables 26 lead to the bar shears 27, back-shear tables 28 and cradles 29. The cooled bars, annealed or not as required, are collected in batches at the delivery sides of the cooling bed 23 and these batches are transferred to the run-out tables 24; all in accordance with usual practice. In case of bars, the rolling of which is completed on the hot mill, the batches thus transferred are conveyed by run-out tables 24 and extension tables 26 for shearing to length on bar shears 27, and the sheared bars are conveyed by back-shear tables 28 to cradles 29 for removal by overhead crane; all in keeping with prevalent practice. By way of example, high carbon spring flats may advantageously be handled in this manner, so also structural and other sections, in case of which accuracy, surface and properties required, are obtainable on the hot mill and the cooling bed.

It will be apparent from the foregoing that by the aid of my invention, products subject to strict tolerances, or of the kind in which superior accuracy is advantageous, such as rounds, by way of example, are produced from rough bars, rolled on a hot mill. After pack-annealing and cooling on the bed 23, the rough rounds are conveyed in batches by run-out tables 24 to the crop shears 25 for removal of any bad ends, at the forward ends of the bars, by cold shearing. The batches are then conveyed by tables 24 and 26 to position alongside transfers 30. By aid of shuffle bars, or other suitable mechanisms, the batches are then moved onto transfers 30 and the rough rounds are fed from there as required, one by one, onto the cold mill approach tables 31. After passing through the cold mills 1 and being converted into rounds of desired accuracy, the individual bars are conveyed by the cold mill run-out tables 33 to position alongside transfers 34. By aid of shuffle-bars or other suitable mechanisms, the finished rounds are moved from the tables 33, collected in batches on transfers 34 and the batches delivered onto tables 26. After shearing on bar shears 27, the finished lengths are conveyed by back shear tables 28 to cradles 29 for further handling in customary manner.

In case of products requiring bright finish, hard surface or particular physical properties, in addition to accuracy, the proceeding is as follows: Rounds of this nature, by way of example, are produced from rough rounds or from blanks, rolled on the hot mill. After pack-annealing and cooling on the bed 23, the rough rounds or blanks are conveyed in batches by run-out tables 24 to the crop shears 25 for removal of any bad ends, at the forward ends of the bars, by cold shearing. The batches are then conveyed by tables 24 and 26 to position alongside the transfers

35. By aid of shuffle bars or other suitable mechanisms, the batches are then moved onto transfers 35. Overhead pickling machines of suitable design remove the batches from the transfers 35 for pickling in troughs 36, washing in troughs 37 and delivery to transfers 38. The time required by the hot mill to roll the rough rounds or blanks which make up the batches provides sufficient time for the picking operations. By 10 aid of shuffle bars or other suitable mechanisms, the pickled and washed rough rounds or blanks are then fed as required, one by one, onto the cold mill approach tables 39. After passing through the cold mills 12 to be converted into 15 rounds of desired finish, physical properties and accuracy, the individual bars are conveyed by the cold mill run-out tables 41 to position alongside transfers 42. By aid of shuffle bars or other suitable mechanisms, the finished rounds are moved 20 from the tables 41, collected in batches on transfers 42 and the batches delivered onto tables 26. After shearing on bar shears 27, the finished lengths are handled same as other finished products already referred to.
25. It will be recognized that not less than two sets of cold rolls are needed to practice my invention. The number of additional sets of rolls required, is determined by the amount of cold work demanded from the mill to achieve desired 30 objectives. If a cold mill be built with sufficient sets of rolls to meet maximum demands, it need only use the number of sets required for any particular purpose. In that case, the rolls of the unused sets are merely opened up to allow free 35 passage for the bars in process. With this idea in view, the theoretical plan shown in Figure 11, has been simplified into the practical and more economical rolling mill layout shown in Figures 12-A and 12-B.
40. Referring now to Figures 12-A and 12-B, a heating furnace 68 is indicated as part of a hot mill designated generally at 69. The hot rolling is completed, either in rolls 70 or in rolls 71, the latter intended principally for coiled products. When the rolls 70 constitute the final pass in the hot mill, then the subsequent sets of hot mill rolls are opened up or removed to allow free 45 passage of products. The hot rolled bars are conveyed by run-in table 72 to a single cooling bed 73 equipped for continuous pack-annealing. Not only does the single cooling bed meet the requirements of the hot mill for capacity, but it affords a much better opportunity for pack-annealing than the double bed, in that all the hot bars go into one continuous pack. They can thus be better annealed and the cost of the cooling bed equipment, an expensive item, is cut in half. The cooled bars, collected at the delivery side of the 50 cooling bed are transferred in batches to the run-out table 74, which can deliver in either of two directions. In case of products the rolling of which may be completed on the hot mill, the batches may be conveyed by run-out table 74 and extension run-out table 75 for shearing on bar shear 76, and the sheared lengths are conveyed by back-shear table 77 for delivery to cradle 78. Every second batch, however, is conveyed by tables 74 and 75 to position alongside transfer 79. 55 by which it is moved onto run-out table 80, leading to bar shear 81. An opening is provided in the frame of the bar shear 76 to allow the batches to pass through on their way to shear 81. The sheared lengths are conveyed by back shear table 82 and delivered to cradle 83. Dou-

ble shearing is thus provided for, notwithstanding the use of a single cooling bed.

In case of products requiring superior accuracy, rough sections of somewhat larger dimensions and of suitable shape are rolled on the hot mill. After pack-annealing and cooling on the bed 73, the rough sections are conveyed in batches by run-out table 74 to the crop shear 84 for removal of any bad ends at the forward ends of the bars. The batches are then conveyed by tables 74 and 75 to position alongside transfers 79 and 85. Batches are moved onto transfer 85, where the bars of the batch are separated to deliver the rough sections, one by one, onto the cold mill approach table 86. The cold mill 87 has several sets of rolls, but preferably only the first two sets are used in cold rolling the rough sections to finished size. The remaining sets of rolls are opened up to allow free passage of the cold rolled bars onto cold mill run-out table 88. Individual bars are thus conveyed to position alongside transfer 89, on which they are collected in batches for transfer to run-out table 75. After shearing, the finished lengths are collected in cradle 78. Every second batch of rough sections arriving alongside transfer 79, however, is moved by this transfer onto run-out table 80, where it remains at rest until it is moved onto transfer 90. There the bars of the batch are separated to deliver the rough sections, one by one, onto the cold mill approach table 91. After passing through the cold mill 92, in the manner described for cold mill 87, the individual cold rolled bars are conveyed on cold mill run-out table 93 to position alongside transfer 94. On it, they are collected in batches for transfer to run-out table 80. After shearing, the finished lengths are collected in cradle 83. Two complete sets of cold-rolling and shearing facilities can thus be operated without interference with one another, to roll and shear products of superior accuracy from rough sections, annealed on a single cooling bed.

Products requiring bright finish, as well as accuracy, are produced from rough sections of somewhat larger dimensions and suitable shape. Products subject to additional cold working, for surface or physical properties, are produced from blanks of proper size and shape, to allow for necessary cold reductions. These rough sections or blanks, rolled on the hot mill 69 and pack-annealed on the cooling bed 73, are delivered in batches on the run-out table 74. Each batch is conveyed to the crop shear 84 for removal of any bad ends at the forward ends of the bars. The direction of travel of the run-out table 74 is then reversed, to convey the batch to the dividing shear 95. If large reductions are called for in the cold mills, it may be necessary to divide the blanks into two or more lengths for cold rolling, in order to limit the finished product to lengths which would be produced were the rolling to be completed on the hot mill. The entire batch of divided cooling bed lengths is conveyed by run-out tables 74 and 96 to position alongside transfer 97. It is moved onto this transfer, successively pickled in troughs 98 and 99 and delivered to transfer table 100. It is conveyed by this transfer table to position alongside the washing trough 101. After washing in this trough, it is delivered to transfer 102 which moves it onto table 103. It is conveyed by this table and the run-out table 80 to position alongside transfers 79 and 85. An opening is provided in the frame of the crop shear 84 to allow the batches to pass through.

A batch of rough sections, or a batch of blanks divided in suitable lengths for cold rolling, may now be moved by transfers 79 and 85 for cold rolling on mill 87. Every second batch, however, is moved by transfer 80 for cold rolling on mill 92. The number of sets of rolls used in the cold rolling operation varies with the amount of cold working to be done and the parts of each divided bar follow one another through the cold mills. The procedure is otherwise the same as already described in cold rolling for accuracy only, until the finished lengths arrive in cradles 78 and 83. Rough sections or blanks, annealed on a single cooling bed, can thus be pickled and fed to two complete sets of cold rolling and shearing facilities; all in a continuous process and without interference between the several operations.

The entire mill layout shown in Figures 12—A and 12—B is preferably housed in suitable buildings, and the pickling equipment is preferably segregated and located in a separate building. Furthermore, the hot rolling, annealing, pickling, cold-rolling and shearing equipment has been duly balanced for capacity of output.

My invention may also be employed for reducing hot-rolled bars to cold-rolled blanks, of great accuracy and very much smaller sectional area, for subsequent annealing or heat treatment and further cold working. By way of example, number five wire rod may thus be produced from, say,  $\frac{3}{8}$ " hot-rolled blanks in the manner illustrated in Figures 13 through 18. Such blanks are preferably finished in the vertical rolls 71 of the hot mill (see Figure 12—A), in the form of 35 pronounced ovals with the major axis vertical, for coiling on reels 108 with vertical spindles, in order to facilitate the coiling of the blank with its major axis throughout the coil maintained in parallel with the spindle of the reel, i. e., the axis 40 of the coil. A limited quantity of such coils may be rolled on the cold mills 87 and 92, particularly by utilizing the time when the hot mill may be rolling finished products, but to handle large tonnages additional cold mills are necessary. In 45 either event, the hot-rolled coils are annealed, handled and transported according to well-known practice. The particular cold mill illustrated in plan view in Figure 13 and the pass reductions, as they are shown in Figures 15 through 18, are predicated on coils such as above referred to, feeding the mill with their axes horizontal.

The oval blank 110 is reduced to rod 111 in rolls 112, 113, 114 and 115, to change the blank coil 116 into rod coil 117. Guides 119, provided immediately ahead of rolls 112, assure proper entry. Controlled tension is maintained in the bar 118 between the several sets of rolls in the manner already explained with reference to cold mill 12. During the rolling operation, the blank coil 116 is retained in position with respect to the mill rolls, on a spindle of suitable construction, and the rod coil 117 is formed on the motor-driven drum of a coiler, at the delivery end of the mill. By controlling the speed of the motor, the bar 118 is subjected to required pull also between the set of rolls 115 and the rod coil 117, to complete the rolling of the rear end under tension. The front end of the bar may pass from rolls 112 to rolls 113 without benefit of tension, but the extreme front end of the rod in finished coil 117 would then be more or less inaccurate. If superior accuracy be demanded throughout the finished coiled length, then the spindle supporting the blank coil 116 must also be controlled as to speed.

Accuracy of wire rods is a matter of well-known importance to subsequent drawing operations, but my new method of cold rolling such rods from hot rolled products of much larger sectional area has other advantages. The ordinary merchant bar mill could thus roll a product of large enough sectional area to be economical and which, by aid of a relatively simple cold mill, could be converted into superior wire rod. An extra annealing operation is required to condition the cold rolled material, but the use of a separate rod mill is obviated. My new method would be particularly advantageous when the required rod tonnage is small.

Although I have described certain preferred applications of my invention, its advantages may be realized in other ways, within the scope of the appended claims.

I claim:

1. In a method of producing metal bars to precise finished dimensions, the steps including hot-rolling bars in cooling-bed lengths which are many times the desired length of the bars, slowly cooling said bars, then subjecting them to cold-rolling in a plurality of passes at least one of which is at an angle to its predecessor, and dividing the bars into desired lengths only after the completion of the cold-rolling.

2. A method as defined by claim 1 characterized by tensioning the lengths during cold rolling sufficiently to limit lateral spread of the metal.

3. A method as defined by claim 1 characterized by decelerating the rolls of one of said passes as the trailing end of a length leaves the preceding pass thereby maintaining tension during the rolling of said end after it has left said last-mentioned pass.

4. In a method of rolling round metal bars of precise finished dimensions, the steps including hot-rolling a blank sufficiently out-of-round to have definite major and minor axes, cooling the blank to cold-rolling temperature, entering the blank in the position of least resistance into a pass formed by parallel rolls, permitting the blank to adjust itself progressively to the position of least resistance, cold-rolling the blank in said pass to reduce the minor axis thereof, entering the blank while it is still in said pass into a pass formed by a second set of rolls, and cold-rolling the blank therein to reduce said major axis.

5. In a method of rolling round metal bars of precise finished dimensions, the steps including hot-rolling a blank sufficiently out-of-round to have definite major and minor axes, cooling the blank to cold-rolling temperature, entering the blank in the position of least resistance into an oval pass formed by a set of parallel rolls, cold-rolling the blank in said pass to reduce the minor axis thereof, entering the blank while it is still in said pass and guided thereby, into a pass formed by a second set of rolls, cold-rolling the blank therein to reduce said major axis, and subjecting the portion of the blank between said sets of rolls to controlled tension.
- 10 6. In a method of rolling round metal bars of precise finished dimensions, the steps including hot-rolling a blank sufficiently out-of-round to have definite major and minor axis, cooling the blank to cold-rolling temperature, progressively gripping the sides of the blank which lie adjacent the ends of the minor axis, entering the blank while it is guided by said gripping action, into a pass formed by parallel rolls, and cold-rolling the blank therein to reduce said major axis.
- 15 7. In a method of producing round metal bars to precise dimensions, the steps including hot-rolling an oval bar with a section having distinctly different major and minor axes and a larger area than that of the desired finished bar, coiling the bar while hot from rolling and slowly cooling it in coiled form, then reducing the section of the bar to circular form by cold-rolling the bar in a plurality of passes under tension sufficient to limit lateral spread of metal under the pressure of the rolls.
- 20 8. In a method of producing round metal bars to precise dimensions, the steps including hot-rolling an oval bar with a section having distinctly different major and minor axes and a larger area than that of the desired finished bars, annealing the bars by slowly cooling them in contact with one another from the hot-rolling temperature, then reducing the section of the bars to circular form by cold-rolling the bars in a plurality of passes under tension sufficient to limit lateral spread of metal under the pressure of the rolls.
- 25 9. In a method of producing round metal bars to precise dimensions, the steps including hot-rolling an oval bar with a section having distinctly different major and minor axes and a larger area than that of the desired finished bars, annealing the bars by slowly cooling them in contact with one another from the hot-rolling temperature, then reducing the section of the bars to circular form by cold-rolling the bars in a plurality of passes under tension sufficient to limit lateral spread of metal under the pressure of the rolls.
- 30 10. In a method of producing round metal bars to precise dimensions, the steps including hot-rolling an oval bar with a section having distinctly different major and minor axes and a larger area than that of the desired finished bars, annealing the bars by slowly cooling them in contact with one another from the hot-rolling temperature, then reducing the section of the bars to circular form by cold-rolling the bars in a plurality of passes under tension sufficient to limit lateral spread of metal under the pressure of the rolls.
- 35 11. In a method of producing round metal bars to precise dimensions, the steps including hot-rolling an oval bar with a section having distinctly different major and minor axes and a larger area than that of the desired finished bars, annealing the bars by slowly cooling them in contact with one another from the hot-rolling temperature, then reducing the section of the bars to circular form by cold-rolling the bars in a plurality of passes under tension sufficient to limit lateral spread of metal under the pressure of the rolls.
- 40 12. In a method of producing round metal bars to precise dimensions, the steps including hot-rolling an oval bar with a section having distinctly different major and minor axes and a larger area than that of the desired finished bars, annealing the bars by slowly cooling them in contact with one another from the hot-rolling temperature, then reducing the section of the bars to circular form by cold-rolling the bars in a plurality of passes under tension sufficient to limit lateral spread of metal under the pressure of the rolls.
- 45 13. In a method of producing round metal bars to precise dimensions, the steps including hot-rolling an oval bar with a section having distinctly different major and minor axes and a larger area than that of the desired finished bars, annealing the bars by slowly cooling them in contact with one another from the hot-rolling temperature, then reducing the section of the bars to circular form by cold-rolling the bars in a plurality of passes under tension sufficient to limit lateral spread of metal under the pressure of the rolls.

GUSTAF L. FISK.